

1

3,278,294

**FERROSILICON AS A DEOXIDIZING, INOCULATING AND/OR ALLOYING AGENT**

Klaus Feldmann, Hermülheim, near Cologne, and Klaus Frank, Knapsack, near Cologne, Germany, assignors to Knapsack - Griesheim Aktiengesellschaft, Knapsack, near Cologne, Germany, a corporation of Germany  
No Drawing. Filed Apr. 11, 1963, Ser. No. 272,197  
Claims priority, application Germany, May 2, 1962,  
K 46,630

8 Claims. (Cl. 75—24)

The present invention relates to an additive of a ferrosilicon alloy suitable for use as a deoxidizing, inoculating and/or alloying agent for increasing the silicon content of steel or cast iron.

It is known that the silicon content of steel or cast iron can be increased by means of crushed or ground commercial ferrosilicon containing 25 to 90% by weight silicon. Ferrosilicon, which preferably contains 75% by weight silicon, can also be used as an inoculating agent in the manufacture of cast iron with spherically separated graphite, the ferrosilicon being added as a germ-forming agent after treatment with magnesium. Independently of the silicon content of the alloy used, the ferrosilicon is employed in lumpy or comminuted form and often in sieved grain fractions having a size, for example, of 0 to 3 mm.; 2 to 6 mm.; 2 to 10 mm.; 3 to 20 mm. or 20 to 40 mm.

Ferrosilicon of such grain size is more especially used:

- (1) As a deoxidizing agent, i.e.,
  - (a) for the deoxidation by precipitation, wherein ferrosilicon is added to the liquid steel to react directly with the oxygen dissolved (in the form of FeO) in the steel with the resultant formation of SiO<sub>2</sub>;
  - (b) for the deoxidation by diffusion, wherein the slag which has formed on the steel bath in the furnace and contains considerable amounts of metal oxides is most frequently reduced with ferrosilicon. The slag is thereby deprived of metal oxides (especially FeO) and thus enabled again to absorb FeO ascending in the steel for the reason that an equilibrium is formed between the FeO-content in the slag and that in the steel, the equilibrium being determined by the FeO-content of the slag, that is to say the proportion of FeO in liquid steel increases as does the FeO-content in the slag;
- (2) As an alloying agent for a plurality of steel grades of which two should be specifically mentioned:
  - (a) dynamo steel and transformer steel
  - (b) heat resistant steels;
- (3) As an alloying agent for increasing the silicon content in cast iron. The ferrosilicon is preferably introduced into the casting pan;

(4) As an inoculating agent in the casting of iron, the ferrosilicon being added to the liquid cast iron shortly before it is being cast which influences the separation of graphite in the manner desired;

(5) As a slag reducing agent. Ferrosilicon may be used as a slag reducing agent even without a deoxidation by diffusion as specified under (1b) above being associated therewith. Ferrosilicon will be used with advantage as a slag reducing agent or as an absolute reducing agent whenever oxides, for example, of chromium, molybdenum, vanadium, tungsten or other high grade metals are intended to be reduced.

It is known, however, that ground ferrosilicon absorbs gases, for example hydrogen during storage. The ferrosilicon is therefore calcined before it is added to steel, the calcination being intended on the one hand to preheat the alloy addition and, on the other, to expell the

2

gases absorbed especially during storage. The gas absorption is a function of the surface area of the ground ferrosilicon grains which appears to indicate that comminuted ferrosilicon contains an increased proportion of gas.

Ground ferrosilicon offers the further disadvantage of being insufficiently stable to abrasion during transport or under any other stress. It may be assumed that during the solidification of ferrosilicon the impurities contained therein crystallize predominantly at the grain boundaries and that the alloy structure therefor exhibits instability to abrasion. The conventional application of crushed and ground ferrosilicon is in most cases burdened with the loss of the finest portions thereof. These are either retained in the slag or are blown away by the thermal buoyancy above the iron melt. Furthermore, these finest ferrosilicon portions undergo favored oxidation as early as they are introduced into the melt bath by the air, which is hot from furnace radiation. Still further, they include a larger proportion of impurities with a reduced content of silicon. It is obvious that the accuracy in the calculation of the ferrosilicon addition for use as an alloying or deoxidizing agent is thereby reduced.

It is also known that lumpy or ground ferrosilicon may decompose by disintegration even without perceivable external influences being observed.

We have now unexpectedly found that ferrosilicon grains having a hard, smooth and rounded-off surface area are free from the disadvantages mentioned above. According to an especially advantageous embodiment of the present invention the ferrosilicon grains have a spherical or globular shape and are surrounded by a thin but gas-impermeable and strongly adhering oxide skin. In addition to the hard grain surface, it is their spherical or globular shape which contributes to a very effective protection against abrasion. The granules having an approximately spherical shape can be used in grain sizes within the limits, for example, of 0.5 to 2 mm.; 2 to 6 mm.; 6 to 10 mm.; or 10 to 25 mm. Grains having a size greater than here indicated often lack the spherical shape, but they are scarcely less abrasion-resistant and gas impermeable.

The grain surface which is smooth, round and enveloped by an oxide film is preferably hardened by chilling as more fully described below, which substantially avoids the separation of impurities at the grain boundaries, with the resultant formation of an alloy having a completely uniform composition. The ferrosilicon particles used in accordance with the present invention therefore do not include segregations such as otherwise observed in ground ferrosilicon as regards the content of silicon and contaminants. Such segregations could result in the addition of ferrosilicon to steel or cast iron failing to produce accurately the predetermined effect.

The ferrosilicon granules used in accordance with the present invention are prepared from the melt in known manner by atomization or spraying. The ferrosilicon melt which may have been prepared, for example, by electrothermal means is atomized or sprayed with the aid of water, steam, air, nitrogen, or the like under a pressure within the range of 1.01 to 13 atmospheres absolute (0.01 to 12 atmospheres gauge).

The atomization of the ferrosilicon melt in known manner with the help of water or steam has previously been burdened with the prejudice that these media could enter into reaction with the melt and thus considerably increase the gas content thereof, especially the hydrogen content thereof, with the resulting granulated ferrosilicon becoming useless for the iron and steel industries. We have now unexpectedly found that the contrary is the case. The atomization by means of water favors immediately a

superficial hardening and the formation of a thin but tight and solidly adhering oxide layer, which avoids any further reaction or diffusion that would be associated with an increase of the gas content. Contrary to all expectation, the ferrosilicon granules obtained from the melt by atomization exhibit at most a hydrogen content the same as the melt before atomization.

In preparing granulated ferrosilicon by atomizing an iron-silicon alloy melt, care should be taken that the resulting granular material is obtained in rather compact form. This is achieved by spraying the liquid iron-silicon melt in a jet not thicker than 40 mm. in diameter and chilling the jet very rapidly to temperatures far below the melting point of iron. Granulated material having a solid massive internal structure should be prepared not only on the ground that compact granular material exhibits a greater stability but also and above all on the ground that hollow and accordingly lighter weight material may be difficult to introduce into steel below the covering slag layer.

Instead of by atomization, the rounded-off ferrosilicon particles can also be prepared in known manner from the melt by directly transforming it into granulated material on a granulating disc, water being here the preferred agent for comminuting the melt and chilling it. The comminuting and/or chilling agents, which include, for example, water, steam, air and nitrogen or the like, are used under a pressure within the range of about 0.01 to 20 atmospheres (gauge pressure) and forced, for example, to pass through nozzles. The granulating step may also be carried out by replacing the disc with a granulating groove. The ferrosilicon melt intended to be atomized or granulated should have a temperature of 1200 to 1600° C.

The granulated ferrosilicon material having a spherical or globular shape and a smooth surface covered by a tight oxide skin which is used in accordance with the present invention as an alloying, inoculating or deoxidizing agent, can also be prepared as follows: the ferrosilicon particles prepared in known manner by grinding solid ferrosilicon are passed in a manner known as such, if desired under pressure and with the aid of an atomizing agent, through a heating zone, for example a flame zone, the ferrosilicon particles being melted round at least superficially on passing that zone and allowed to solidify in a cooling or chilling zone following the heating zone.

Granulated ferrosilicon material which has been prepared with the use of water or steam as the atomizing agent or with the use of water as the chilling agent, should be dried in known manner. The drying should take place at temperatures which are not too high so as to ensure that the oxide skin formed on the individual ferrosilicon particles is not substantially enlarged but merely strengthened. The material may be subjected, for example, to a direct continuous current drying process, wherein the hottest temperature is produced at those places where the ferrosilicon is moist. The continuous current drying ensures that the individual grains are heated to a temperature not exceeding 1000° C. Care should also be taken during the drying step that heating or drying gases are used

in which the partial pressure of steam is fairly low. Thus, it is of advantage to use very pure carbon monoxide (more than 90% CO) as the heating gas. This process can be carried out in the manner described above as a calcining drying process at relatively high temperatures. Alternatively, the material may be dried, for example, by indirect heating at relatively low temperatures, for example, at 120 to 200° C., but in this event the oxide skin is only slightly strengthened.

As already mentioned above, the granulated ferrosilicon particles used in accordance with the present invention offer the particular advantage of having a thin and tightly adhering oxide skin which in conjunction with their hardened surface does not permit the subsequent absorption of gas.

In other words, the ferrosilicon particles retain their initial gas content which emanates from the melt without the gas content being ultimately increased due to the external influences during storage. The advantage offered thereby is outstanding and obvious. Thus, the ferrosilicon can be used immediately in a manner independent from storage and without being subjected to an additional calcining step for alloying, inoculating or deoxidizing purposes. In granulated material, which has been prepared from ferrosilicon degassed, for example, by treating it in *vacuo*, this low hydrogen content is retained. The risk of gas bubbles being formed in the melt by the addition of ferrosilicon containing too high a proportion of gas, which in most cases has been absorbed during storage and which is not expelled during calcination, is therefore substantially reduced. In other words, the use of granulated ferrosilicon having a smooth and hardened surface does no longer result in the steel quality being specifically impaired by the formation of so-called flakes due to the hydrogen contained in the ferrosilicon material.

We have also found that granulated ferrosilicon material having a spherical shape and a smooth, hardened surface when used in particles of identical size with a defined surface area, undergoes dissolution at a uniform rate. This uniform rate of dissolution and the uniform distribution of the silicon content and of the inevitable impurities over any ferrosilicon particle enable an extensive automatic control in the iron and steel-producing industries. The rates of dissolution and hence the effects produced by the ferrosilicon added, which differ in each particular application, can be determined beforehand and, since they always take place at the same velocity and with the same efficiency the automatic control adapted thereto.

The following tests were conducted to establish the advantages offered by granulated ferrosilicon obtained by atomizing a ferrosilicon melt.

(1) 600 kg. of a ferrosilicon charge of 2060 kg. were granulated with the aid of an annular nozzle under a vapor pressure of 0.5 atmosphere (gauge pressure) to a grain size of 1 to 10 mm., while 1460 kg. solidified ferrosilicon were crushed and then ground to particles of identical size.

TABLE 1

| Grade                           | Grain size in mm. |       |      |      |      |      |         |
|---------------------------------|-------------------|-------|------|------|------|------|---------|
|                                 | 0-0.5             | 0.5-1 | 1-2  | 2-4  | 4-6  | 6-8  | Above 8 |
| Crushed or ground ferrosilicon: |                   |       |      |      |      |      |         |
| Portion of grain, percent.....  | 26.0              | 19.5  | 14.5 | 12.0 | 9.2  | 8.3  | 11.0    |
| Si, percent.....                | 69.8              | 71.13 | 72.9 | 73.0 | 74.3 | 74.6 | 75.7    |
| Al, percent.....                | 1.30              | 1.13  | 0.92 | 0.85 | 0.81 | 0.73 | 0.68    |
| Oxides, percent.....            | 2.1               | 0.9   | 0.9  | 0.8  | 0.8  | 0.75 | 0.7     |
| Granulated ferrosilicon:        |                   |       |      |      |      |      |         |
| Portion of grain, percent.....  | 2.5               | 6.5   | 7.0  | 32.8 | 27.2 | 15.1 | 10.9    |
| Si, percent.....                | 73.2              | 72.9  | 73.4 | 73.1 | 73.1 | 73.5 | 73.0    |
| Al, percent.....                | 0.97              | 0.95  | 0.90 | 0.92 | 0.89 | 0.91 | 0.92    |
| Oxides, percent.....            | 2.5               | 1.6   | 1.6  | 1.3  | 1.3  | 1.2  | 1.2     |

The above Table 1 clearly indicates the uniformity of the silicon content in all grain sizes and the uniform distribution of the impurities, identified in the above table by the aluminum content, inasmuch as the granulated material prepared by atomizing molten ferrosilicon is concerned, and it also indicates the corresponding non-uniformity inasmuch as the crushed and ground ferrosilicon in concerned.

The data indicated for the oxide film are confirmed by the determination of the total oxides. It can readily be seen that the oxide content of granulated ferrosilicon is only slightly greater than that of the crushed or ground ferrosilicon.

(2) The resistance to abrasion of granulated ferrosilicon as compared with that of crushed ferrosilicon was determined by exposing 50 grams of either material in a ball mill under identical conditions to grinding stress. The data obtained represent merely comparative values. The resistance to abrasion was determined by determining the proportion of grains which had been ground after 1, 2, 3 and 4 minutes, respectively, under such heavy stress to a grain size of less than 0.5 mm.

TABLE 2

| Initial grain size | Grade                | Portion of grains in percent of material used—grinding time in min. |      |      |      | Composition, percent |      |
|--------------------|----------------------|---------------------------------------------------------------------|------|------|------|----------------------|------|
|                    |                      | 1                                                                   | 2    | 3    | 4    | Si                   | Al   |
| 0.5-2.0 mm-----    | Granulated FeSi----- | 2.0                                                                 | 3.2  | 5.2  | 7.8  | 73.1                 | 0.92 |
|                    | Crushed FeSi-----    | 28.6                                                                | 44.8 | 48.6 | 62.6 | 72.0                 | 1.05 |
| 2.0-4.0 mm-----    | Granulated FeSi----- | 1.8                                                                 | 3.4  | 5.2  | 7.4  | 73.1                 | 0.92 |
|                    | Crushed FeSi-----    | 24.6                                                                | 30.0 | 40.0 | 48.6 | 73.0                 | 0.85 |

Of the granulated material which had been chilled and therefore had a hardened surface and a globular shape only as little as 7.8 or 7.4% had been comminuted after 4 minutes of grinding to a grain size of less than 0.5 mm., whereas 62.6 or 48.6% of the crushed ferrosilicon had been comminuted to a grain size of less than 0.5 mm.

(3) The stability of the granulated material to outdoor influences for example during storage, was tested by placing 10 grams each of granulated ferrosilicon and of crushed ferrosilicon in water at 90° C. and measuring the gas evolved. Absolute values again were not obtained. The test results indicate, however, to the expert the superior resistance to chemical reactions and/or diffusion phenomena of water or steam of the granulated material as opposed to the crushed material.

TABLE 3

|                      | Grain size, mm. | Evolution of gas in cc. after— |        |        |
|----------------------|-----------------|--------------------------------|--------|--------|
|                      |                 | 2 hrs.                         | 4 hrs. | 6 hrs. |
| Granulated FeSi----- | 0.5-2           | 0.6                            | 0.6    | 0.8    |
|                      | 2-4             | 0.6                            | 0.6    | 0.8    |
| Crushed FeSi-----    | 0.5-2           | 2.4                            | 4.3    | 5.4    |
|                      | 2-4             | 2.2                            | 3.5    | 5.0    |

The present invention provides more particularly an additive of ferrosilicon suitable for use as a deoxidizing, inoculating and/or alloying agent for increasing the silicon content in steel or cast iron, the additive consisting of granulated ferrosilicon having a smooth and rounded-off, preferably a globular shape and a hard surface produced by chilling. The granulated ferrosilicon is preferably surrounded by an oxide skin and has a massive internal structure.

The ferrosilicon additive generally contains 25 to 90% by weight, preferably 70 to 80% by weight, silicon and it is used in grain sizes within the range of about 0.5 to about 25 mm. in diameter.

The granulated ferrosilicon additive is prepared by atomizing or spraying a ferrosilicon melt, which may have been produced, for example, by electrothermal means, with the aid of water, steam, air, nitrogen or the like under a pressure within the range of 0.01 to 12 atmospheres (gauge pressure), or by directly granulating the ferrosilicon melt on a granulating disc, the agents used for comminuting and/or chilling the melt, which include water, steam, air, nitrogen and the like, being employed under a pressure within the range of between 0.01 and 20 atmospheres (gauge pressure) and being forced, for example, to pass through nozzles.

The ferrosilicon melt may also be transformed into granulated form by granulating it in a granulating groove.

The ferrosilicon melt to be comminuted should have a temperature of about 1200 to 1600° C. and it should be degassed in known manner, for example, by treatment in vacuo before it is transformed into granular form by atomization or granulation.

The resulting granulated ferrosilicon is then freed from adhering water by subjecting it to a calcining drying step.

According to a further feature of the present invention

the granulated ferrosilicon is prepared by grinding solid ferrosilicon which is subsequently passed, if desired under pressure and with the aid of an atomizing agent through a heating zone, for example a flame zone, the ferrosilicon particles being melted round at least superficially on passing that zone and allowed to solidify in a cooling or chilling zone following the heating zone.

The following examples serves to illustrate the invention, but it is not intended to limit the invention thereto.

#### Example

The reduction of slag may serve as an example to describe the advantage offered by the granulated ferrosilicon having a smooth and rounded-off, preferably a globular shape and a surface area hardened by chilling as compared with ground ferrosilicon.

Slag was reduced as usual while using ferrosilicon, 75% having a grain size within the limits of 0 to 3 mm. This small grain size had to be used in order to achieve a good distribution of the ferrosilicon over the slag surface area. Under identical conditions, the slag of 20 charges was treated (a) with ground ferrosilicon and (b) with granulated ferrosilicon having the above indicated grain size and composition.

Altogether 1050 kg. ground ferrosilicon were necessary for slag reduction, whereas merely 880 kg. granulated ferrosilicon were required to produce the same effect.

The silicon content in the ground ferrosilicon had been determined as being 74.5% and the silicon content in the granulated ferrosilicon had been determined as being 73.9%. In other words, 1050 kg. ground ferrosilicon corresponding to 782 kg. silicon and 880 kg. granulated ferrosilicon corresponding to 650 kg. silicon had been consumed, respectively.

The degree to which the silicon was utilized had thus been improved by about 20%.

We claim:

75 1. A method of deoxidizing liquid steel which com-

prises adding to said liquid steel a deoxidizing agent comprising abrasion resistant, granulated ferrosilicon particles of substantially uniform chemical composition, said particles containing from more than 25 to 90 percent by weight silicon, having a massive internal structure, a smooth and rounded off surface area hardened by chilling, a grain size within the limits of about 0.5 to about 25 mm. and being enveloped by a gas-impermeable oxide film whereby the particles are resistant to absorbing gas during storage rendering it unnecessary to preheat them prior to use to expel such gas.

2. A method of inoculating cast iron for influencing the separation of graphite which comprises adding to the liquid cast iron shortly before casting an inoculating agent comprising abrasion resistant, granulated ferrosilicon particles of substantially uniform chemical composition, said particles containing from more than 25 to 90 percent by weight silicon, having a massive internal structure, a smooth and rounded off surface area hardened by chilling, a grain size within the limits of about 0.5 to about 25 mm. and being enveloped by a gas-impermeable oxide film whereby the particles are resistant to absorbing gas during storage rendering it unnecessary to preheat them prior to use to expel such gas.

3. A method of increasing the silicon content of an alloy selected from the group consisting of cast iron and steel which comprises adding to the liquid alloy an alloying agent comprising abrasion resistant, granulated ferrosilicon particles of substantially uniform chemical composition, said particles containing from more than 25 to 90 percent by weight silicon, having a massive internal structure, a smooth and rounded off surface area hardened by chilling, a grain size within the limits of about 0.5 to about 25 mm. and being enveloped by a gas-impermeable oxide film whereby the particles are resistant to absorbing gas during storage rendering it unnecessary to preheat them prior to use to expel such gas.

4. A method of reducing the metal oxide content of slag which comprises adding to the liquid slag a slag reducing agent comprising abrasion resistant, granulated

5

10

15

20

25

30

35

40

ferrosilicon particles of substantially uniform chemical composition, said particles containing from more than 25 to 90 percent by weight silicon, having a massive internal structure, a smooth and rounded off surface area hardened by chilling, a grain size within the limits of about 0.5 to about 25 mm. and being enveloped by a gas-impermeable oxide film whereby the particles are resistant to absorbing gas during storage rendering it unnecessary to preheat them prior to use to expel such gas.

5. A method according to claim 1 wherein the granulated ferrosilicon particles contain 70 to 80 percent by weight silicon.

6. A method according to claim 2 wherein the granulated ferrosilicon particles contain 70 to 80 percent by weight silicon.

7. A method according to claim 3 wherein the granulated ferrosilicon particles contain 70 to 80 percent by weight silicon.

8. A method according to claim 4 wherein the granulated ferrosilicon particles contain 70 to 80 percent by weight silicon.

#### References Cited by the Examiner

##### UNITED STATES PATENTS

1,942,173 5/1932 Justheim ----- 75-57  
2,144,200 6/1939 Rohn ----- 75-57 X  
2,527,186 10/1950 Griffiths ----- 75-57

##### FOREIGN PATENTS

777,775 6/1957 Great Britain.  
798,269 7/1958 Great Britain.

##### OTHER REFERENCES

Alloy Cast Irons Handbook, second edition 1944, American Foundrymen's Association, p. 37.  
Metals Handbook, 1948 edition, American Society for Met., pp. 338 and 515.

DAVID L. RECK, Primary Examiner.

P. WEINSTEIN, Assistant Examiner.